# EUROPEAN PATENT SPECIFICATION

(11) **EP 0 211 968 B1**
(45) Date of publication and mention of the grant of the patent: **28.02.1990**
(21) Application number: 85109591.9
(22) Date of filing: 30.07.1985
(51) Int. Cl.: B41M 5/26

(54) **Heat-sensitive recording material**
Wärmeempfindliches Aufzeichnungsmaterial
Matériel pour l'enregistrement sensible à la chaleur

(43) Date of publication of application: 04.03.1987
(73) Proprietor: SANYO KOKUSAKU PULP CO. LTD., Chiyoda-ku Tokyo 100 (JP)
(72) Inventor: Kasamatsu, Norikazu, Kawasaki-shi Kanagawa-ken (JP); Matsukawa, Masao, Setagaya-ku Tokyo (JP); Hirata, Hirokazu, Kamifukuoka-shi Saitama-ken (JP); Mishima, Masaru, Nerima-ku Tokyo (JP)
(74) Representative: Müller-Boré & Partner Patentanwälte

(56) References cited:
- FR-A- 2 417 396
- FR-A- 2 542 261
- US-A- 3 560 229
- PATENT ABSTRACTS OF JAPAN, vol. 9, no. 25 (M-355)[1748], 2nd February 1985, page 36 M 355
- PATENT ABSTRACTS OF JAPAN, vol. 7, no. 265 (M-258)[1410], 25th November 1983, page 116 M 258
- PATENT ABSTRACTS OF JAPAN, vol. 8, no. 37 (M-277)[1474], 17th February 1984, page 71 M 277
- PATENT ABSTRACTS OF JAPAN, vol. 5, no. 139 (M-86)[811], 3rd September 1981
- PATENT ABSTRACTS OF JAPAN, vol. 5, no. 187 (M-98)[859], 26th November 1981, page 58 M 98
- PATENT ABSTRACTS OF JAPAN, vol. 6, no. 48 (M-119)[926], 27th March 1982
- PATENT ABSTRACTS OF JAPAN, vol. 7, nr. 221 (M-246)[1366], 30th September 1983
- PATENT ABSTRACTS OF JAPAN, vol. 7, no. 223 (M-247)[1368], 4th October 1983
- PATENT ABSTRACTS OF JAPAN, vol. 6, no. 220 (M-169)[1098], 5th November 1982
- PATENT ABSTRACTS OF JAPAN, vol. 6, no. 228 (M-171)[1106], 13th November 1982

## Description

### FIELD OF THE INVENTION

The present invention relates to a heat-sensitive recording material which is good in environmental stability and, more particularly, it relates to a heat-sensitive recording paper for self-adhesive labels which has no protective layer.

### BACKGROUND OF THE INVENTION

Hitherto, heat-sensitive recording papers have been used as a heat-sensitive recording type, self-adhesive label.

In the case of such a heat-sensitive recording type, self-adhesive label, when pasticizers present in plastic films, such as dioctyl adipate (DOA) and dioctyl phthalate (DOP), penetrate into a heat-sensitive, color-forming layer, there was found a problem of decolorization of the printed portion (color-formed portion). Accordingly, it cannot be used as a self-adhesive label for plasticizer-containing plastic wrapping film. Further, when water or oils penetrate into the heat-sensitive, color-forming layer, the printed image smears or the image density reduces with a lapse of time. Moreover, in the case that the printing is carried out by bringing the heat-sensitive, color-forming layer into direct contact with a thermal head, if the amount of a binder present in the heat-sensitive, color-forming layer is too high, the residue build-up and sticking readily occur. Accordingly, in order to prevent such occurrence, the amount of the binder in the heat-sensitive, color-forming layer is necessarily reduced, which, however, leads to a drawback that the surface strength is weak. Thus, in the case that the printing is carried out on the surface of the heat-sensitive, color-forming layer, the heat-sensitive, color-forming layer is entrained in the rubber roll side, whereby the printing is no longer possible.

In order to remove the above drawbacks, an attempt to not only prevent the transver and penetration of plasticizers, water and oils into the heat-sensitive, color-forming layer but also impart it with a surface strength has hitherto been made by providing a protective layer on the heat-sensitive, color-forming layer for the purpose of adapting such a heat-sensitive recording material to self-adhesive labels.

As a main component of the protective layer, there are used water-soluble high molecular weight compounds such as, for example, polyvinyl alcohol or modified products thereof, starch or modified products thereof, etc.

However, in the case of the conventional heat-sensitive recording type, self-adhesive labels having a protective layer mainly composed of a water-soluble high molecular weight compound, though the decolorization of the printed portion by plasticizers and the surface strength are improved, there may occur the transfer and penetration of water and oils from the edge portions and back side of the label, resulting in decolorization of the printed portion by water and oils. Further, by providing the protective layer on the heat-sensitive, color-forming layer, when the color formation is carried out by means of a thermal head, there occur problems that the heat responsibility reduces and the color formation sensitivity lowers. Still further, because of the increase of a production step for providing the protective layer, there is a disadvantage of cost increase.

### SUMMARY OF THE INVENTION

An object of the present invention is to provide a heat-sensitive recording material which can overcome the above-described drawbacks of the conventional techniques and which can not only prevent the decolorization of the color-formed image by plasticizers, water and oils but also be produced at a low manufacturing cost.

In order to achieve the above object, the present inventors have made extensive investigations and found that this object can be attained by a heat-sensitive recording material comprising a heat-sensitive, color-forming layer containing as color-forming components a colorless or pale-colored leuco dye and an acidic compound capable of allowing the leuco dye to color develop by heating, wherein a color former comprising a specified fluoran derivative, a developer comprising a specified sulfone compound, and a binder comprising a specified high molecular weight compound are combined with each other, which finding accomplished the present invention.

That is, the present invention is to provide a heat-sensitive recording material comprising a support having on one surface thereof a heat-sensitive, color-forming layer comprising a color former comprising a fluoran derivative represented by the following general formula (I): wherein Rᵢ and R₂ each represents a lower alkyl group, and X represents a halogen atom, a lower alkyl group, a cyano group, or a nitro group, a developer comprising bis(p-hydroxyphenyl)sulfone or a derivative thereof represented by the following general formula (II): wherein R₃ and R₄ each represents a hydrogen atom, an alkyl group, an aryl group, an alkoxy group, a phenoxy group, a carbonyl group, a nitro group, or a cyano group, and a binder comprising an ammonium salt of a diisobutylene/maleic anhydride copolymer and a styrene/butadiene copolymer, wherein in the amount of said styrene/butadiene copolymer in said binder is from 0,5 to 1.0 parts by weight based on parts by weight of said ammonium salt of diisobutylene/maleic anhydride copolymer the styrene content of which is 58 to 62 mol%.

In the heat-sensitive recording material according to the present invention, the printing or recording of images can be carried out on one side of the support in a heating manner, and when a self-adhesive layer is provided on the other side of the support, the heat-sensitive recording material can be used as various price labels, measuring labels, name plates, seals, etc.

### DETAILED DESCRIPTION OF THE INVENTION

Examples of the fluoran derivative represented by the above-described general formula (I) include 3- dibutylamino-7-o-chloroanilinofluoran, 3-dibutylamino-7-o-fluoroanilinofluoran, 3-diethylamino-7-o-chloroanilinofluoran, and 3-diethylamino-7-o-fluoroanilinofluoran, with 3-dibutylamino-7-o-fluoroanilino- fluoran being particularly preferred.

The color former represented by the general formula (I) which is used in the present invention can be used in combination with other color formers.

Specific examples of the compound represented by the general formula (II) include bis(p-hydroxyphenyl)sulfone, bis(3-aryl-4-hydroxyphenyl)sulfone, bis(2,5-dimethyl-4-hydroxy)sulfone, bis(2,5-diethyl-4-hydroxy)sulfone, bis(2,5-dipropyl-4-hydroxy)sulfone, bis(2,5-dibutyl-4-hydroxy)sulfone, bis(2,5-dibenzyl-4-hydroxy)sulfone, bis(2,5-dimethoxy-4-hydroxy)sulfone, bis(2,5-diethoxy-4-hydroxy)sulfone, bis(2,5-dipropoxy-4-hydroxy)sulfone, bis(2,5-dibutoxy-4-hydroxy)sulfone, bis(2,5-diphenoxy-4-hydroxyphenyl)sulfone, bis(2,5-dibenzyloxy-4-hydroxyphenyl)sulfone, bis(2,5-dimethoxycarbonyl-4-hydroxyphenyl)sulfone, bis(2,5-diethoxycarbonyl-4-hydroxyphenyl)sulfone, bis(2,5-diacetyl-4-hydroxyphenyl)sulfone, bis(2,5-dibenzoyl-4-hydroxyphenyl)sulfone, bis(4-hydroxy-3-nitro)su)fone, bis(3-cyano-4-hydroxy)sulfone, 5-ethyl-4-hydroxy-2-methylphenyl 4'-hydroxy-2'-methoxy-5'-methylphenyl sulfone, 5'-ethoxy-4-hydroxy-2-methylphenyl 5'-ethyl-2'-ethoxy-4'-hydroxyphenyl sulfone, and 5-benzyloxy-4-hydroxy-2-methylphenyl 4'-hydroxy-2'-methoxy-5'-methylphenyl sulfone.

The developer represented by the general formula (II) which is used in the present invention is known per se from JP-A 59 169 887 and can be used in combination with other developers.

According to the above-described combination of the color former with the developer, the plasticizer resistance, water resistance and oil resistance are improved to a considerable extent, but when brought into contact with a plastic film containing a plasticizer, water or an oil for a long period of time, there was observed a tendency of decolorization of the color-formed portion. Further, the surface strength of the heat-sensitive, color-forming layer is still weak, and even though in order to improve the surface strength, a styrene/butadiene copolymer used in coated paper was applied as a binder, the residue build-up and sticking occurred.

In order to improve these points, the present inventors have made further extensive investigations and found that such an object can be obtained by using, as a binder for the heat-sensitive, color-forming layer, an ammonium salt of a diisobutylene/maleic anhydride copolymer (preferably one mol of a diisobutylene group being reacted with one mol of a maleic anhydride group) represented by the following general formula (III): wherein Rs represents an diisobutylene group together with a styrene/butadiene copolymer (the styrene content being from 58 to 62 mol%) represented by the following general formula (IV):

As the ammonium salt of diisobutylene/maleic anhydride copolymer used as the binder in the present invention, those having a molecular weight of from 10,000 to 200,000 are suitable, and one having one mol of an isobutylene group bonded to one mol of a maleic anhydride group is known per se from JP-A 58 193 187 and JP-A 59 169 887 and is particularly effective for improving the preservability. Further, the styrene/butadiene copolymer has an effect for improving the surface strength of the heat-sensitive, color-forming layer, and one having a styrene content of from 58 to 62 mol% is effective for the improvement in surface strength of the heat-sensitive, color-forming layer. If the styrene content is too high, the heat-sensitive, color-forming layer becomes rigid to cause a reduction in surface strength, whereas if the butadiene content is too high, the residue build-up and sticking readily occur upon printing by means of a thermal head.

With respect to the binder, a combination use of the ammonium salt of diisobutylene/maleic anhydride copolymer with the styrene/butadiene copolymer is essential in the present invention. If only the ammonium salt of diisobutylene/maleic anhydride copolymer is used, the surface strength of the heat-sensitive, color-forming layer is low, whereas if only the styrene/butadiene copolymer is used, the plasticizer resistance is low and the residue build-up and sticking readily occur.

From 0.5 to 1.0 part by weight of the styrene/butadiene copolymer is mixed with one part by weight of the ammonium salt of diisobutylene/maleic anhydride copolymer. Further, the binder of the present invention can be used in combination with other binders such as polyvinyl alcohol, hydroxyethyl cellulose, carboxymethyl cellulose, starch, etc.

The heat-sensitive, color-forming layer of the present invention can be formed by known methods. As the support, a sheet-like material, such as paper, synthetic paper or plastic films, can be used. Onto one side of the support is coated a coating solution containing the above-described fluoran derivative, bis(p-hydroxyphenyl)sulfone and binder, to thereby form a heat-sensitive, color-forming layer.

If desired, the heat-sensitive, color-forming layer can contain known auxiliary additives such as fine white pigments such as calcium carbonate, talc, clay, silica, titanium oxide, and urea/formalin resin, and heat-fusible substances such as various waxes, higher fatty acid metal salts, and higher fatty acid amides, to thereby improve the sharpness of the color-formed image.

On the other hand, on the other side of the support is provided a pressure-sensitive adhesive layer by known methods such that it can be adhered to plastic films or wrapping paper, and a release substrate is laminated to the back side thereof. There can be thus obtained a heat-sensitive recording type, self-adhesive label.

The thus obtained heat-sensitive recording material according to the present invention excels in recording properties and environmental stability of the heat-sensitive, color-forming layer, without residue build-up and sticking during the printing. Furthermore, the heat-sensitive recording type self-adhesive label obtained by applying a pressure-sensitive adhesive onto the back side of the support using the heat-sensitive recording material of the present invention is more excellent than ever.

The present invention will now be explained in more detail with reference to the examples, but it is to be understood that the invention is not limited thereto.

### EXAMPLE 1

The following components were mixed together for 24 hours in a ball mill to prepare dispersions A and B.

The dispersions A and B were mixed together with as a binder a mixture of 6 parts by weight of a 20% diisobutylene/maleic anhydride copolymer ammonium salt aqueous solution (molecular weight: about 50,000) and 1.6 parts by weight of a 50% styrene/butadiene copolymer latex (molar percentage of styrene: 58 to 62%), and the mixture was coated on one side of wood free paper (basis weight: 50 g/m²) and then dried to form a heat-sensitive, color-forming layer. There was thus obtained a heat-sensitive recording material according to the present invention.

### EXAMPLE 2

The following components were mixed together for 24 hours in a ball mill to prepare dispersions A and B.

The dispersions A and B were mixed together with as a binder a mixture of 6 parts by weight of a 20% diisobutylene/maleic anhydride copolymer ammonium salt aqueous solution (molecular weight: about 50,000) and 1.6 parts by weight of a 50% styrene/butadiene copolymer latex (molar percentage of styrene: 58 to 62%), and the mixture was coated on one side of wood free paper (basis weight: 50 g/m²) and then dried to form a heat-sensitive, color-forming layer. There was thus obtained a heat-sensitive recording material according to the present invention.

### COMPARATIVE EXAMPLE 1

Heat-sensitive recording materials 1-A and 1-B for comparison were obtained in the same manner as in Example 1 except that the 3-dibutylamino-7-o-fluoro^{q}nilinofluoran used in the dispersion A was replaced by 3-diethylamino-7-p-chloroanilinofluoran and 3-(N-methyl-N-cyclohexylamino)-6-methyl-7-anilino- fluoran, respectively.

### COMPARATIVE EXAMPLE 2

A heat-sensitive recording material for comparison was obtained in the same manner as in Example 1 except that the bis(p-hydroxyphenyl)sulfone used in the dispersion B was replaced by 4,4'-isopropylidene diphenol.

### COMPARATIVE EXAMPLE 3

A heat-sensitive recording material for comparison was obtained in the same manner as in Example 1 except that 10 parts by weight of a 20% diisobutylene/maleic anhydride copolymer ammonium salt aqueous solution was used as the binder.

### COMPARATIVE EXAMPLE 4

A heat-sensitive recording material for comparison was obtained in the same manner as in Example 1 except that 4 parts by weight of a 50% styrene/butadiene copolymer latex was used as the binder.

### COMPARATIVE EXAMPLE 5

A heat-sensitive recording material for comparison was obtained in the same manner as in Example 1 except that a mixture of 2.5 parts by weight of a 20% diisobutylene/maleic anhydride copolymer ammonium salt aqueous solution and 3 parts by weight of a 50% styrene/butadiene copolymer latex was used as the binder.

On the back side of each of the heat-sensitive recording materials was laminated a silicone resin- coated release paper having thereon an acrylic-based pressure-sensitive adhesive layer at a coverage of 20 g/m², through the pressure-sensitive adhesive layer, and the laminate was cut off into a suitable size to obtain a heat-sensitive self-adhesive label.

The thus obtained seven heat-sensitive self-adhesive labels were printed by means of a label printer (HP-9303, made by Tokyo Denki K.K.), whereby a color formation test, a residue build-up and sticking test, a environmental stability test, and a surface strength test were carried out.

The results are shown in the following table.

Each of the tests was carried out in the following manner.

### Color Density

The color formation was carried out by printing by means of a label printer, and the color-formed portion was measured by a Macbeth densitometer RD-514. (Hereinafter, the densities were all measured by the Macbeth densitometer RD-514.)

### Background Density

The density of the background portion was measured.

### Plasticizer Resistance

A portion which had been subjected to color formation by printing by means of the label printer was covered by a soft polyvinyl chloride film and after standing at room temperature for 24 hours, the density thereof was measured.

### Water Resistance

A portion which had been subjected to color formation by printing by means of the label printer was dipped in water at room temperature for 24 hours, and the density thereof was then measured.

### Oil Resistance

A portion which had been subjected to color formation by printing by means of the label printer was applied with a sesame oil, and after standing at room temperature for 24 hours, the density thereof was measured.

### Surface Strength

The heat-sensitive recording material was printed with an ultraviolet light-curable ink (made by Toka Shikiso K.K.) by means of an RI tester (Akashi Seisakusho Co., Ltd.), and the transfer amount of the heat-sensitive, color-forming layer to the rubber roll side was observed.

It is clear from the above table that the heat-sensitive recording material according to the present invention Example 1 and 2 is of such a high quality that it is excellent in color formation, has a high whiteness in the background portion, is so good in environmental stability that the color does not disappear by the plasticizer, water, and oil, and is printable and free from residue build-up and sticking. On the other hand, in Comparative Examples 1-A and 2, the printed portion was decolorized by the plasticizer, oil and water and became unreadable; in Comparative Example 1-B, the background density was high as 0.25 and the image of the label was markedly reduced; in Comparative Example 3, although the density of the printed portion after the preservation test by the plasticizer, oil and water was 1.10 or more and a sharp image was kept, the surface strength was quite unsatisfactory; and in Comparative Examples 4 and 5, the printed portion was decolorized by the plasticizer and caused the residue build-up and sticking, and the recording materials cannot be put into practical use.

## Claims

A heat-sensitive recording material comprising a support having thereon a heat-sensitive, color-forming layer mainly composed of as color-forming components a colorless or pale-colored leuco dye and an acidic compound capable of allowing said leuco dye to color develop by heating, wherein said heat-sensitive, color-forming layer comprises a color former comprising a fluoran derivative represented by the following general formula (I): wherein R₁ and R₂ each represents a lower alkyl group, and X represents a halogen atom, a lower alkyl group, a cyano group, or a nitro group, a developer comprising bis(p-hydroxyphenyl)sulfone or a derivative thereof represented by the following general formula (II): wherein Rₛ and R₄ each represents a hydrogen atom, an alkyl group, an aryl group, and alkoxy group, a phenoxy group, a carbonyl group, a nitro group, or a cyano group, and a binder comprising an ammonium salt of a diisobutylene/maleic anhydride copolymer and a styrene/butadiene copolymer, wherein the amount of said styrene/butadiene copolymer in said binder is from 0.5 to 1.0 parts by weight based on the parts by weight of the ammonium salt of diisobutylene/maleic anhydride copolymer the styrene content of which is 58 to 62 mol%.

## Patentansprüche

Wärmeempfindliches Aufzeichnungsmaterial aus einem Träger mit einer wärmeempfindlichen farbbildenden Schicht, die sich hauptsächlich aus einem farblosen oder hellgefärbten Leukofarbstoff als farbbildende Komponenten und einer sauren Verbindung zusammensetzt, die dazu in der Lage ist, den Leukofarbstoff durch Erhitzen zu einer Farbe zu entwickeln, wobei die wärmeempfindliche farbbildende Schicht einen Farbbildner aus einem Fluoranderivat der folgenden allgemeinen Formel (I) aufweist, worin R₁ und R₂ jeweils eine niedere Alkylgruppe bedeuten und X ein Halogenatom, eine niedere Alkylgruppe, eine Cyanogruppe oder eine Nitrogruppe ist, ein Entwickler ein Bis(p-hydroxyphenyl)sulfon oder ein Derivat davon der folgenden allgemeinen Formel (11) aufweist, wobei R₃ und R₄ jeweils ein Wasserstoffatom, eine Alkylgruppe, eine Arylgruppe, eine Alkoxygruppe, eine Phenoxygruppe, eine Carbonylgruppe, eine Nitrogruppe oder eine Cyanogruppe bedeuten, und ein Bindemittel aus einem Ammoniumsalz aus einem Diisobutylen/Maleinsäureanhydrid-Copolymeren und einem Styrol/Butadien-Copolymeren vorgesehen ist, wobei die Menge des Styrol/Butadien-Copolymeren in dem Bindemittel 0,5 bis 1,0 Gewichtsteile, bezogen auf die Gewichtsteile des Ammoniumsalzes des Dilsobutylen/Maleinsäureanhydrid-Copolymeren beträgt und der Styrolgehalt 58 bis 62 Mol-% ausmacht.

## Revendications

Matériau d'enregistrement thermosensible comprenant un support recouvert d'une couche thermosensible développant une coloration, composée principalement, en tant que composants développant une coloration, d'un leuco-colorant incolore ou de couleur pâle et d'un composé acide à même de permettre audit leuco-colorant de développer une coloration par chauffage, dans lequel ladite couche thermosensible développant une coloration comprend un générateur de couleur comportant un dérivé de fluora- ne représenté par la formule générale (I) suivante: dans laquelle Rᵢ et R₂ représentent chacun un groupe alkyle inférieur et X représente un atome d'halogène, un groupe alkyle inférieur, un groupe cyano, ou un groupe nitro, un développeur comprenant de la bis(p-hydroxyphényl)sulfone ou un de ses dérivés représentés par la formule générale (11) suivante: dans laquelle Rₐ et R₄ représentent chacun un atome d'hydrogène, un groupe alkyle, un groupe aryle, un groupe alkoxy, un groupe phénoxy, un groupe carbonyle, un groupe nitro, ou un groupe cyano, et un liant comprenant un sel d'ammonium d'un copolymère diisobutytène/anhydride maléique et un copolymère styrène/butadiène dans lequel la quantité dudit copolymère styrène/butadiène dans ledit liant est de 0,5 et 1,0 partie en poids par rapport à la partie en poids du sel d'ammonium du copolymère diisobutylè- ne/anhydride maléique, et dont la teneur en styrène est de 58 à 62 moles %.
